

## UNITED STATES PATENT OFFICE

2,115,852

## AZO DYES

Chester W. Hannum and Swanie S. Rossander,  
Wilmington, Del., assignors to E. I. du Pont de  
Nemours & Company, Wilmington, Del., a  
corporation of Delaware

No Drawing. Application July 8, 1937,  
Serial No. 152,527

## 4 Claims. (Cl. 8—5)

This invention relates to blue and violet dyes of the azo class and to means of producing and applying them.

- The prior art discloses blue and violet dyes of a type bearing a superficial similarity to the dyes of this invention. In German Patent 163,321 (1905), for example, are dyes which have fair utility but are lacking in sufficient fastness to washing, whereby the utility is greatly diminished. 5 It is an object of this invention to produce new dyes of blue and violet shades which have exceptional fastness to washing and which are also fast to light, heat, chlorine, and the other influences which affect the permanence of dyes. 10 The objects of the invention are attained, generally speaking, by manufacturing and applying to the fiber by development thereon the class of colors represented by the formula: 15



- 20 in which aryl is one of the group consisting of benzene and alpha-naphthylamine and in which at least one "aryl" has a water-solubilizing substituent, E has a single nucleus from the group consisting of benzene and phenyl-pyrazolone, 35 Z has a single nucleus from the group consisting of beta-naphthol, phenyl-pyrazolone, meta-tolylene-diamine, and acetoacet-arylide, and Y is one or more of the group consisting of hydrogen, alkyl, alkoxy, halogen, carboxy, and sulfonic acid. 40 The dye is applied to the fiber by direct dyeing

with a dyestuff represented in the form of its free acid by the formula:



in which aryl is one of the group consisting of benzene and alpha-naphthylamine, at least one of the said aryls having a water-solubilizing group from the class consisting of carboxylic acid and sulfonic acid, E is one of the group consisting of benzene and phenyl-pyrazolone, having a free amino group, and Y is at least one of the group consisting of hydrogen, alkyl, alkoxy, and halogen, diazotizing and developing with beta-naphthol, preferably, or with phenyl-pyrazolone, acetoacet-arylide, and meta-tolylene-diamine, or with a benzene or naphthalene compound capable of coupling. 10

The following examples illustrate the invention but do not limit it.

## Example I

25 Five parts of cotton piece goods are dyed in the usual manner known to those in the art with four hundredths part of H-acid->alpha-naphthylamine->1,6-Cleves acid->cresidine. The dyed fabric (blue in shade) is rinsed in cold water and put in a casserole with 200 parts of water at 20° C. Add three-tenths part of sodium nitrite and four-tenths part of sulfuric acid. Stir 15 minutes. Rinse with cold water. Dissolve one-tenth part of 2-naphthol in 200 parts of water and one-twentieth part of caustic soda. Stir the solution rapidly while adding the above rinsed piece goods. Stir for 15 minutes. Rinse in cold water and dry. The dyeing is a blue shade. The probable formula of the dye on the fiber is: 30



| Ex. | Diazo component                                                                                     | Coupling component             | Shade on cellulose |
|-----|-----------------------------------------------------------------------------------------------------|--------------------------------|--------------------|
| 5   |                                                                                                     |                                |                    |
| 2   | H-acid → alpha-naphthylamine → 1,6-Cleves acid → cresidine                                          | Beta-naphthol                  | Blue.              |
| 3   | do                                                                                                  | 1-phenyl-3-methyl-5-pyrazolone | Violet.            |
| 4   | do                                                                                                  | Acetosacet-anilide             | Do.                |
| 5   | do                                                                                                  | Meta-tolylene diamine          | Blue.              |
| 10  |                                                                                                     |                                |                    |
| 6   | H-acid → alpha-naphthylamine → 1,7-Cleves acid → cresidine                                          | Beta naphthol                  | Do.                |
| 7   | H-acid → alpha-naphthylamine → mixed Cleves acid → cresidine                                        | do                             | Do.                |
| 8   | H-acid → alpha-naphthylamine → 1,6-Cleves acid → meta toluidine                                     | do                             | Do.                |
| 9   | H-acid → alpha-naphthylamine → 1,6-Cleves acid → para-xylidine                                      | do                             | Do.                |
| 15  |                                                                                                     |                                |                    |
| 10  | H-acid → alpha-naphthylamine → mixed Cleves acid → acetyl-methoxyphenylene-diamine                  | do                             | Do.                |
| 11  | H-acid → alpha-naphthylamine → 1,7-Cleves acid → para-xylidine                                      | do                             | Do.                |
| 12  | H-acid → cresidine → 1,7-Cleves acid → cresidine                                                    | do                             | Do.                |
| 13  | H-acid → alpha-naphthylamine → 1,6-Cleves acid → cresidine                                          | do                             | Do.                |
| 20  |                                                                                                     |                                |                    |
| 14  | H-acid → 1,6-Cleves acid → 1,6-Cleves acid → cresidine                                              | do                             | Do.                |
| 15  | H-acid → alpha-naphthylamine → 1,6-Cleves acid → 1-meta-amino-phenyl-5-pyrazolone-3-carboxylic acid | do                             | Do.                |
| 16  | H-acid → alpha-naphthylamine → 1,6-Cleves acid → 1-meta-amino-phenyl-3-methyl-5-pyrazolone          | do                             | Do.                |
| 17  | 1-amino-8-naphthol-4,6-disulfonic acid → alpha-naphthylamine → 1,6-Cleves acid → cresidine          | do                             | Do.                |
| 18  | 1-amino-8-naphthol-3,6-disulfonic acid → alpha-naphthylamine → 1,6-Cleves acid → cresidine          | do                             | Do.                |
| 25  |                                                                                                     |                                |                    |

In the foregoing table the arrows mean coupled by the diazo reaction.

30 These colors have excellent shades of blue and violet and outstanding fastness to washing and outstanding discharge properties. They are also fast to the usual destructive influences and accordingly are superior colors.

At least one of the center nuclei must contain a water-solubilizing group, such as sulfonic or carboxylic acid and two such groups are often of assistance. Each of the aryl nuclei may also contain one or more substituents from the group consisting of hydrogen, halogen, alkyl, alkoxy, carboxy, and sulfonic acid.

As many apparently widely different embodiments of this invention may be made without departing from the spirit and scope thereof, it is to be understood that we do not limit ourselves to the specific embodiments thereof except as defined in the appended claims.

We claim:  
1. The compound represented in the form of  
its sodium salt by the formula:  
50

nucleus from the group consisting of benzene and phenyl pyrazolone, Z has a single nucleus from the group consisting of beta-naphthol, 1-phenyl-3-methyl-5-pyrazolone, meta-tolylene diamine, acetoacet-arylide, and Y is one or more of the group consisting of hydrogen, alkyl, alkoxy, halogen, carboxy, and sulfonic acid.

3. The compound represented in the form of its free acid by the formula:



in which aryl is one of the group consisting of benzene and alpha naphthylamine and in which at least one "aryl" has a water-solubilizing substituent, E has a single nucleus from the group consisting of benzene and phenyl-pyrazolone, Z has a single nucleus from the group consisting of



2. The compound represented in the form of its free acid by the formula:

beta-naphthol, phenyl-pyrazolone, meta-tolyl-ene-diamine, and acetoacet-arylide, and Y is one



in which aryl is one of a group consisting of benzene and alpha-naphthylamine, E has a single

or more of the group consisting of hydrogen, alkyl, alkoxy, halogen, carboxy, and sulfonic acid.

4. The process which comprises dyeing cellulose with a compound represented in the form of its free acid by the formula:



group from the class consisting of carboxylic acid and sulfonic acid, E is one of the group consisting of benzene and phenyl pyrazolone, having a free amino group, and Y is at least one of the group consisting of hydrogen, alkyl, alkoxy, and halogen, diazotizing the color on the fiber, and coupling it to one of a group of compounds consisting of beta-naphthol, 1-phenyl-3-methyl-5-pyrazolone, meta-tolylene-diamine and acetoacet-arylide.

5

10

CHESTER W. HANNUM.  
SWANIE S. ROSSANDER.